

1

2,982,729

**HIGH TEMPERATURE LUBRICATING GREASE  
CONTAINING A p,p'-DIAMINODIPHENYL-  
ETHER**

Henryk A. Cyba, Chicago, and Ralph B. Thompson, Hinsdale, Ill., assignors, by mesne assignments, to Universal Oil Products Company, Des Plaines, Ill., a corporation of Delaware

No Drawing. Filed Apr. 2, 1958, Ser. No. 725,808

7 Claims. (Cl. 252—40.7)

This invention relates to high temperature lubricating grease of improved stability for use under the more severe conditions of modern technology. This application is a continuation-in-part of copending application Serial No. 545,513, filed November 7, 1955 and now abandoned.

During recent years developments in aircrafts, turbines, automobiles, trucks, farm equipment, railroad equipment, industrial machinery, etc. have resulted in equipment operating at higher temperatures, higher speeds and greater loads. These developments have presented new problems in the satisfactory lubrication of such equipment and require lubricating greases which will be effective under these more severe conditions. Greases previously available were found wanting because of instability at the higher temperatures.

The new problems presented by these developments are illustrated, for example, in the turbo jet engines, where satisfactory lubrication is required at temperatures ranging from as low as  $-65^{\circ}$  F. and as high as  $275^{\circ}$  F. during use. Temperatures up to  $500^{\circ}$  F. are encountered at intervals of from one to two hours during shutdown. New developments in winter grade crank case oils, aviation instruments, automatic weapons, etc. are additional examples of recent developments which have presented new problems in lubrication. As hereinbefore set forth, there is a great need for lubricating greases which are stable during use under these severe conditions. In addition, these greases should be useable for longer times and, therefore, improved stability is essential.

In accordance with the present invention, improved stability is imparted to lubricating grease by incorporating therein an inhibitor of specific configuration. As will be illustrated in the appended examples, the inhibitors of the present invention appear to be peculiarly advantageous in lubricating greases and particularly during use at high temperatures, high speeds and with greater loads. In contrast thereto, it will be noted that similar but different additives do not impart this high stability to the lubricating grease.

The high temperature lubricating greases of the present invention generally include lithium base grease, sodium base grease, potassium base grease, barium base grease, strontium base grease, aluminum base grease, beryllium base grease, cadmium base grease, magnesium base grease, lead soap grease, complex soap grease, etc., or mixtures known as mixed base greases including barium-calcium, barium-lithium, sodium-calcium, sodium-barium, aluminum-lithium, lithium-strontium, etc.

2

These greases are solid or semi-solid gels and in general are prepared by the addition to mineral oils of hydrocarbon-soluble metal soaps or salts of higher fatty acids as, for example, lithium stearate, calcium stearate, aluminum naphthenate, etc. In another method, the metal soap or salt is added to synthetic oils including, for example, di-(2-ethylhexyl) sebacate or azelate, di-tetradecyl sebacate, tricresyl phosphate, polyalkylene oxides, silicones, alkyl or alkyaryl polysiloxanes or blends of these with petroleum oil. The grease may contain thickening agents such as silica, Bentonite, carbon black, polyacrylates, talc, polyamides, alkylureas, phthalocyanines, etc. Another type of grease is prepared from oxidized petroleum wax to which the saponifiable base is combined with the proper amount of the desired saponifying agent, and the resultant mixture processed to produce a grease.

While the present invention is particularly applicable to the greases specified above, it is understood that the 20 novel method of the present invention may be utilized for the stabilization of other greases including whale grease, wool grease, etc., and those made from inedible fats, tallow, butcher's wastes, etc.

In one embodiment the present invention relates to a 25 method of stabilizing a high temperature lubricating grease which comprises incorporating therein a stabilizing concentration of a p,p'-diaminodiphenyl ether inhibitor.

In a specific embodiment the present invention relates 30 to a method of stabilizing a high temperature lithium base lubricating grease which comprises incorporating therein from about 0.001% to about 5% by weight of p,p'-diaminodiphenyl ether.

In another specific embodiment the present invention 35 relates to a method of stabilizing a high temperature calcium base lubricating grease which comprises incorporating therein from about 0.001% to about 5% by weight of p,p'-diisopropylaminodiphenyl ether.

In still another embodiment the present invention 40 relates to a high temperature lubricating grease containing a stabilizing concentration of the inhibitor herein set forth.

As hereinbefore set forth, the diaminodiphenyl ether 45 of the present invention appears to be peculiarly effective in imparting high stability to lubricating greases and particularly such greases for use at high temperature, high speed and with greater loading. In addition to protecting the grease from normal deterioration encountered at these conditions, the inhibitor of the present invention also serves to deactivate or passivate the effect of metals contained in or contacted by the grease. In many cases such metals tend to catalyze oxidation and other undesirable deterioration of the grease. However, this undesirable effect is offset by the novel inhibitors 50 of the present invention.

In one embodiment, the inhibitor of the present invention comprises p,p'-diaminodiphenyl ether. In another embodiment, the inhibitor comprises a p,p'-dialkylaminodiphenyl ether. In the latter embodiment, it generally is preferred that the alkyl groups are of secondary configuration; that is, the alkyl group is attached to the nitrogen atom at an intermediate carbon atom of the alkyl group. Illustrative compounds in this class include p,p'-diisopropylaminodiphenyl ether, p,p'-di-sec-butyl-

aminodiphenyl ether, p,p'-di-sec-amylaminodiphenyl ether, p,p'-di-sec-hexylaminodiphenyl ether, p,p'-di-sec-heptylaminodiphenyl ether, p,p'-di-sec-octylaminodiphenyl ether, p,p'-di-sec-nonylaminodiphenyl ether, p,p'-di-sec-decylaminodiphenyl ether, p,p'-di-sec-undecylaminodiphenyl ether, p,p'-di-sec-dodecylaminodiphenyl ether, p,p'-di-sec-tetradecylaminodiphenyl ether, p,p'-di-sec-penta-decylaminodiphenyl ether, p,p'-di-sec-hexadecylaminodiphenyl ether, p,p'-di-sec-heptadecylaminodiphenyl ether, p,p'-di-sec-octadecylaminodiphenyl ether, p,p'-di-sec-nonadecylaminodiphenyl ether, p,p'-di-sec-eicosylaminodiphenyl ether, etc.

While compounds containing secondary alkyl groups are preferred, it is understood that suitable compounds containing n-alkyl substituents may be employed, but not necessarily with equivalent results. Illustrative compounds in this class include p,p'-dimethylaminodiphenyl ether, p,p'-diethylaminodiphenyl ether, p,p'-di-n-propylaminodiphenyl ether, p,p'-di-n-butylaminodiphenyl ether, p,p'-di-n-amyloaminodiphenyl ether, p,p'-di-n-hexylaminodiphenyl ether, p,p'-di-n-heptylaminodiphenyl ether, p,p'-di-n-octylaminodiphenyl ether, p,p'-di-n-nonylaminodiphenyl ether, p,p'-di-n-decylaminodiphenyl ether, p,p'-di-n-undecylaminodiphenyl ether, p,p'-di-n-dodecylaminodiphenyl ether, etc.

In general it is preferred that the inhibitor comprises a symmetrical compound; that is, the alkyl groups are of the same configuration and chain length. However, in some cases the alkyl groups may be different in either the number of carbon atoms or in the configuration thereof, or both, and preferably are selected from the alkyl groups hereinbefore specifically set forth. In another embodiment the hydrocarbon radicals attached to the nitrogen atoms may comprise alkenyl groups as, for example, in compounds such as p,p'-dipropenylaminodiphenyl ether, p,p'-dibutylaminodiphenyl ether, p,p'-dipentenylaminodiphenyl ether, p,p'-dihexenylaminodiphenyl ether, p,p'-di-heptenylaminodiphenyl ether, p,p'-dioctenylaminodiphenyl ether, etc., which alkenyl groups preferably are of secondary configuration.

From the above description, it will be noted that a number of different inhibitor compounds may be used in accordance with the present invention. However, it is understood that the different compounds are not necessarily equivalent. The specific compound to be used will depend upon the availability and/or cost of preparation and also upon the effectiveness in the particular grease to be stabilized. It is understood that a mixture of compounds may be employed, the particular compounds preferably being selected from those hereinbefore specifically set forth. In some cases, a mixture of isomers is produced during the manufacture of the inhibitor and, when desired, the mixture is used as such, thereby avoiding the additional time and expense of separating the components of the mixture.

In general, the inhibitor is utilized in a concentration of from about 0.001% to about 5% by weight of the grease, although in some cases higher or lower concentrations may be employed. The exact concentration to be used will depend upon the particular grease being treated. In most cases a concentration of from about 0.01% to about 3% by weight generally is employed.

It is understood that the inhibitor may be used along with other additives incorporated in grease, including higher alcohols, esters, organic amines, polybutene, sulfurized fatty materials, sulfur chloride compounds, dyes, perfumed materials, fillers, etc. In some cases, it may be of advantage to also include an additional metal deactivator as, for example, disalicyl diamino propane, ethylene diamine tetra-acetic acid or the tetrasodium salt thereof, etc., or to include other additives such as tricresyl phosphate, trialkyl phenols, including 2,6-di-tert-butyl-4-methylphenol, 2,4-di-methyl-6-tert-butyl-phenol, alkylated diphenyl amines, phenyl naphthyl amines, di-

alkyl phenylene diamines, phenothiazine, organic selenium compounds, etc., as well as corrosion inhibitors, extreme pressure additives, viscosity index improvers, etc. When desired, the inhibitor of the present invention may be prepared as a mixture with one or more of these other additives and incorporated in this manner in the grease or components thereof.

The inhibitor of the present invention may be incorporated in the grease in any suitable manner and at any suitable stage of preparation. Thus, it may be added to one or more components of the grease prior to compositing and processing thereof or it may be added to the mix at any time, preferably before final processing in order to obtain intimate mixing and dissolving of the inhibitor in the grease.

The following examples are introduced to illustrate further the novelty and utility of the present invention but not with the intention of unduly limiting the same.

#### EXAMPLE I

Calcium base grease is prepared by the following general method. The calcium soap is prepared by mixing the fat, hydrated lime equivalent to about one-seventh of the fat, mineral oil sufficient to make about one-fourth of the total charge, and about 0.5% of water. The ingredients are mixed and heated to about 140° F. and then dry lime is added, agitation and heat continued until saponification is completed. Additional oil then is added and the mixture heated to 220-230° F. Additional oil is added to bring the mixture to the desired consistency, and then is heated at 170-180° F. At this stage, 1% by weight of p,p'-di-sec-butylaminodiphenyl ether, along with other additives, dyes, etc. is added, and the mixing is continued until formation of grease of the desired structure.

#### EXAMPLE II

p,p'-diaminodiphenyl ether was utilized as an inhibitor in a lithium grease. The grease was prepared by mixing 91% of a highly refined Pennsylvania oil having a Saybolt viscosity of 180 second at 100° F. with 8% of lithium stearate. The mixture was heated to about 450° F. while agitating the same. Subsequently, the grease was cooled to 320° F. while agitating and, at this temperature, 1% of p,p'-diaminodiphenyl ether was added. Agitation was continued and the mixture was allowed to cool to about 250° F., and the grease then further cooled slowly to room temperature.

The stability of the grease was tested according to a modified Norma Hoffman method, in which a sample of the grease is placed in a bomb in the presence of brass discs acting as an oxidation catalyst and oxygen is charged thereto. The bomb then is heated to 212° F., and the time required for a drop of 5 pounds pressure is taken as the induction period. In this run, a control sample of the grease (not containing this additive) had an induction period of 4 hours. On the other hand, a sample of the grease containing 1% by weight of p,p'-diaminodiphenyl ether had an induction period of 187 hours. Thus, it will be noted that the inhibitor of the present invention was exceptionally effective in improving the stability of the grease.

#### EXAMPLE III

The inhibitor used in this example is p,p'-diisopropylamino diphenyl ether. When incorporated in a concentration of 1% by weight to another sample of the grease described in Example II and tested in the same manner, the inhibitor of this example served to increase the induction period of the grease from 4 hours to 133 hours. Here again, it will be noted that the inhibitor of the present invention served to stabilize the grease to a considerable extent.

#### EXAMPLE IV

As hereinbefore set forth, the diaminodiphenyl ether

of the present invention appears to be particularly adapted for use in high temperature lubricating grease. The evaluations of the greases in Examples II and III were conducted at a temperature of 212° F. Because these greases are required for use at higher temperatures, the following examples report evaluations made at 250° F. and according to ASTM Method D-942. The grease used in this example was a lithium base grease containing 8% by weight of lithium stearate and a mineral oil. The results of these evaluations are reported in the following table:

Table I

| Inhibitor                                               | Induction period<br>(Hours to 5<br>pounds pressure<br>drop) |
|---------------------------------------------------------|-------------------------------------------------------------|
| None                                                    | 2                                                           |
| 0.3% by weight of p,p'-diaminodiphenyl ether            | 21.5                                                        |
| 0.3% by weight of p,p'-diisopropylaminodiphenyl ether   | 200                                                         |
| 0.3% by weight of p,p'-tetramethylaminodiphenyl methane | 9                                                           |

From the data in the above example it will be noted that the diaminodiphenyl ethers were very effective in improving the stability of the grease at the high temperature. In contrast, the diaminodiphenyl methane was substantially of no value. This demonstrates the unique properties of the diaminodiphenyl ether to impart high stability to the lubricating grease in contrast to the absence of this property in the diaminodiphenyl methane, even though the latter may be said to be of similar chemical configuration to the diaminodiphenyl ether.

## EXAMPLE V

This example reports additional evaluations in a different lithium base grease than reported in Example IV. The lithium base grease also contained 8% by weight of lithium stearate but was prepared with a different mineral oil. When evaluated under the same conditions as reported in Example IV, the following data were obtained.

Table II

| Inhibitor                                             | Induction period<br>(Hours to 5<br>pounds pressure<br>drop) |
|-------------------------------------------------------|-------------------------------------------------------------|
| None                                                  | 4                                                           |
| 0.1% by weight of p,p'-diaminodiphenyl ether          | 54                                                          |
| 0.3% by weight of p,p'-diaminodiphenyl ether          | 142                                                         |
| 1% by weight of p,p'-tetramethylaminodiphenyl methane | 39                                                          |

Here again, the peculiar properties of the diaminodiphenyl ether in high temperature grease is demonstrated. It will be noted that three-tenths the concentration of diaminodiphenyl ether yielded a grease having the stability of more than three times that obtained with the diaminodiphenyl methane. Even the use of one-tenth as much diaminodiphenyl ether still produced a grease of higher stability than that obtained by using 1% by weight of diaminodiphenyl methane.

## EXAMPLE VI

As demonstrated by Examples IV and V, the diaminodiphenyl ethers impart high stability to the greases evaluated at the higher temperature. This effect is peculiar to the diaminodiphenyl ethers and is not obtained with diaminodiphenyl methanes. While this improvement at high temperatures is extremely important for the reasons hereinbefore set forth, the following data show that the diaminodiphenyl ethers are considerably more effective than the diaminodiphenyl methanes even when evaluated at the lower temperature of 210° F. and in the presence of a brass catalyst. These evaluations were made with an 8% lithium base grease prepared from a heavy min-

75

eral oil, and the evaluations were made in the same manner as described in Example II.

Table III

| Inhibitor                                              | Induction period<br>(Hours to 5<br>pounds pressure<br>drop) |
|--------------------------------------------------------|-------------------------------------------------------------|
| None                                                   | 8                                                           |
| 1% by weight of p,p'-diaminodiphenyl ether             | >93                                                         |
| 1% by weight of p,p'-di-sec-butylaminodiphenyl methane | 22                                                          |
| 1% by weight of p,p'-diethylaminodiphenyl methane      | 27                                                          |
| 1% by weight of p,p'-dibenzylaminotriphenyl methane    | 23                                                          |

10 From the data in the above table, it will be noted that the diaminodiphenyl ether is many times more effective than the diaminodiphenyl methanes and the diaminotriphenyl methane shown in the above table.

15 The data in the above examples demonstrate the peculiar effectiveness of the diaminodiphenyl ethers to impart high stability to lubricating greases. This effectiveness is especially important to lubricating greases when used at high temperatures. These improved results are 20 outstanding, particularly when compared with the lack of effectiveness of the diphenyl methanes at these high temperatures. Furthermore, as seen from the data in Example VI, the superiority of the diphenyl ethers also is evidenced even when the grease is evaluated at the lower temperature.

25 30 We claim as our invention:

35 1. A lubricating grease composition consisting essentially of a major amount of a lubricating oil, a grease-thickening amount of a metal soap of a higher fatty acid and a stabilizing concentration of a p,p'-diaminodiphenyl ether.

40 2. A lubricating grease composition consisting essentially of a major amount of a lubricating oil, a grease-thickening amount of a metal soap of a higher fatty acid and from about 0.001% to about 5% by weight of p,p'-diaminodiphenyl ether.

45 3. A lubricating grease composition consisting essentially of a major amount of a lubricating oil, a grease-thickening amount of a metal soap of a higher fatty acid and from about 0.001% to about 5% by weight of a p,p'-dialkylaminodiphenyl ether.

50 4. A lubricating grease composition consisting essentially of a major amount of a lubricating oil, a grease-thickening amount of a lithium soap of a higher fatty acid and from about 0.01% to about 3% by weight of p,p'-diisopropylaminodiphenyl ether.

55 5. A lubricating grease composition consisting essentially of a major amount of a lubricating oil, a grease-thickening amount of a lithium soap of a higher fatty acid and from about 0.01% to about 3% by weight of p,p'-di-sec-butylaminodiphenyl ether.

60 6. A lubricating grease composition consisting essentially of a major amount of a lubricating oil, a grease-thickening amount of a calcium soap of a higher fatty acid and from about 0.01% to about 3% by weight of p,p'-diisopropylaminodiphenyl ether.

65 7. A lubricating grease composition consisting essentially of a major amount of a lubricating oil, a grease-thickening amount of a calcium soap of a higher fatty acid and from about 0.01% to about 3% by weight of p,p'-di-sec-butylaminodiphenyl ether.

## References Cited in the file of this patent

## UNITED STATES PATENTS

|              |                   |               |
|--------------|-------------------|---------------|
| 70 2,290,860 | Burk et al. _____ | July 28, 1942 |
| 2,346,356    | Burk _____        | Apr. 11, 1944 |
| 2,367,264    | Burk et al. _____ | Jan. 16, 1945 |
| 2,440,530    | Yates _____       | Apr. 27, 1948 |
| 2,443,026    | Detwiler _____    | June 8, 1948  |
| 2,910,437    | Symon _____       | Oct. 27, 1959 |